

## UNITED STATES PATENT OFFICE

1,931,108

## DISCHARGE PRINTING

Frederick Baxter Downing, Carneys Point, N. J., and Richard G. Clarkson, Wilmington, Del., assignors to E. I. du Pont de Nemours & Company, Wilmington, Del., a corporation of Delaware

No Drawing. Application December 29, 1930  
Serial No. 505,464

19 Claims. (Cl. 8—5)

This invention relates to the art of textile printing and more particularly to the discharged dyed style of printing upon the cellulose ester and ether type of artificial silk. It specifically contemplates the utilization of organic thiocyanates as swelling agents for cellulose acetate textile material.

There is a type of textile printing known as the "discharged dyed style". In general this process comprises dyeing the fabric throughout and thereafter printing on certain portions or areas thereof what is known as a "discharge paste". This paste is a composition comprising some substance or substances capable of removing, destroying or permanently decoloring the dye already affixed to the fabric. Upon suitable aftertreatment the color is removed at the places in contact with the discharge paste.

There is a modification of this process known as "color discharge printing" which is generally the same as the process above described except that the "discharge paste" comprises another dye so that upon discharge of the original dye from the dyed fabric the second dye (that is, the dye in the discharge paste) remains on the discharged portion. As will be obvious the second dye is of a type which is not adversely affected by the color discharging materials present in the paste.

It is known that the dyeing of cellulose acetate and the like is a different phenomena from the dyeing of other fibers. Cellulose acetate is dyed by reason of the formation of the solid solution of the dyestuff in the fiber. The dyeing of other fibers results from the adsorption of minute particles of the dyestuff upon the surface of the fiber (Brandenberger Textiliber 10, 215, 461: 1929).

The ordinary reduction discharge methods at present in general use for the production of discharge effects upon silk, wool and cotton materials are based upon the use of sodium formaldehyde-sulfoxylate as a discharging agent. These methods are ineffective when applied to the cellulose acetate type of fiber. Heretofore, in the discharging of cellulose acetate dyeings it has been found necessary to use a different discharging agent or to add to the paste containing the ordinary discharge agent a substance which will swell the fiber and permit its penetration by the reducing or decoloring agent. The materials used for swelling the fiber are commonly known as "swelling agents".

As an example of the first of the two procedures noted, mention may be made of the disclosure by

Fischesser (U. S. Patent 1,747,540 of Feb. 18, 1930) relating to neutral zinc sulfoxylate as a discharging agent.

In the second of the above procedures, the swelling agents heretofore known and used are such compounds as triacetin, cyclo-hexanone and ethylene glycol. Recently Smith (U. S. Patent 1,651,639 of Dec. 6, 1929) has proposed ammonium sulfo-cyanide, calcium sulfo-cyanide and barium sulfo-cyanide as swelling agents. With many dyes, however, even with use of these sulfo-cyanides the reduction has been insufficiently complete to be commercially practical.

This invention has as an object the provision of a method for producing clear and white discharges upon fabrics composed wholly or in part of cellulose esters or ethers. Further objects are the production of discharges upon fabrics of cellulose derivatives of dyes which have not heretofore been dischargeable, the provision of new color discharge printing processes and effects on cellulose esters or ethers, the provision of new reusterling processes for cellulose esters or ethers, and in general an advancement of the art. Other object will appear hereinafter.

These objects are accomplished by the present invention according to which organic thiocyanates are incorporated in discharge printing pastes. The invention will be readily understood from a consideration of the following examples and description in which the parts are given by weight.

## Discharge printing paste

Twenty (20) parts of sodium formaldehyde sulfoxylate were dissolved in 55 parts of gum tragacanth solution containing 60 parts of gum tragacanth in one thousand parts of water and when the sulfoxylate was in complete solution 25 parts of a guanidine thiocyanate solution of approximately 50% by weight strength was added.

## Example I

A fabric composed of cellulose acetate was dyed in the customary manner with Ionamine A powder, diazotized, developed with beta-oxy-naphthoic-acid and was afterwards printed with the discharge printing paste described above. After the fabric had been printed it was aged for 3-5 minutes in an ordinary type of rapid ager at 100° C. It was then washed in water at 60° C. for 3 minutes and dried. A pure white discharge was obtained.

When the above procedure was repeated with the substitution of 25 parts of a 50% ammonium sulfocyanide solution for the 25 parts of guani-

dine thiocyanate solution the dyestuff of the printed design was only slightly affected. The discharge was very incomplete.

*Example II*

5 A fabric composed of cellulose acetate was dyed with 1-methyl-4-amino-5-methoxy-benzene-azo-4'-benzamid in the customary manner and was afterwards diazotized and coupled with beta-naphthol in the customary manner. It was then printed and afterwards treated as described in Example I. The discharge obtained by the use of guanidine thiocyanate was a clear white, whereas that obtained by the use of ammonium sulfo-cyanide was of a yellowish cast.

*Example III*

20 Material composed of cellulose acetate was dyed in the customary manner with Cibacete diazo black B and was afterwards diazotized and coupled with beta-oxy-naphthoic acid in the customary manner. The material was then printed and afterwards treated as described in Example I. A complete discharge of slightly yellowish tone was obtained by the use of guanidine thiocyanate whereas the use of ammonium sulfo-cyanide produces no appreciable discharge effect.

*Example IV*

25 Material composed of cellulose acetate was dyed in the customary manner with Celitazol AZ and was afterwards diazotized and coupled with beta-oxy-naphthoic acid in the customary manner. The material was then printed with a color discharge printing paste made up as follows:

30 Fifteen (15) parts by weight of British gum was dissolved in 24 parts of gum tragacanth solution containing 60 parts of gum tragacanth in one thousand parts of water by heating. Twenty (20) parts of sodium formaldehyde sulfoxylate was then dissolved in this thickener and afterwards 15 parts diethylene glycol, 10 parts guanidine thiocyanate and 6 parts of sodium hydroxide solution containing 300 parts of sodium hydroxide in 700 parts of water were added.

35 The resulting paste was then cooled and when cold 10 parts of Ponsol brilliant green G paste (dimethoxy-dibenzanthrone) was added and uniformly mixed in by stirring.

40 After the fabric had been printed it was aged for 3-5 minutes in an ordinary type of rapid ager at 100° C. It was then washed in water at 60° C. and dried. A brilliant green print on a black ground was obtained.

45 When the above procedure was repeated with the substitution of 10 parts of ammonium sulfo-cyanide for the 10 parts of guanidine thiocyanate, the shade of the printed design was much duller and weaker.

50 In the discharge paste above described, potassium or other alkali metal formaldehyde-sulfoxylates may be used if desired.

55 The amount of guanidine thiocyanate to be added to the discharge paste for the production of satisfactory discharges varies so widely that definite limits cannot be given. The amount to be used depends upon the nature of the fabric, the size of the filaments, the nature of the dye-stuffs employed, the strength of the dyeing and the like. No general rule can therefore be laid down as to the concentration of the reagent to be employed. For each specific case this may be readily determined by experiment by one skilled in the art.

60 Variations in the discharging conditions may be made if desired.

Preferably the guanidine thiocyanate is added to the various compositions mentioned in the form of its aqueous solution.

65 When guanidine thiocyanate is employed as the swelling agent a part of the beneficial effects obtained are undoubtedly due to the presence of the guanidine radical. This is shown by the fact that discharges are produced by the use of this reagent which are unobtainable by the use of an equal weight of ammonium sulfocyanide. This is true in spite of the fact that a given quantity of ammonium sulfocyanide contains 50% more of the sulfocyanide (thiocyanate) radical than an equal amount of guanidine thiocyanate.

70 Guanidine thiocyanate may also be used as a printing assistant in color printing on acetyl cellulose and other cellulose esters and ethers. It is, in addition, a valuable relustering agent for these materials.

75 Numerous advantages of the invention are outstanding. Among these may be mentioned

(1) The production of discharges of a character unobtainable by previously known methods. This is especially true on more difficultly dischargeable colors such as those of the examples.

(2) The production of white discharges of superior stability. The samples of Example II were retained and after one week the ammonium sulfo-cyanide discharge had a strong yellow cast whereas the guanidine thiocyanate had not appreciably changed.

(3) The production of discharge areas which are whiter than those produced by discharge paste not containing guanidine thiocyanate. This is clearly shown by the results of the process of Example II.

80 As many apparently widely different embodiments of this invention may be made without departing from the spirit and scope thereof, it is to be understood that we do not limit ourselves to the specific embodiments thereof except as defined in the appended claims.

We claim:

1. The process which comprises printing a discharge composition containing guanidine thiocyanate on dyed cellulose acetate material and finishing the discharge operation by ageing at about 100° C., washing and drying.

2. The production of discharge effects on acetyl cellulose materials which comprises the addition of guanidine thiocyanates to an alkali metal formaldehyde-sulfoxylate discharge printing paste.

3. The production of color discharge effects on acetyl cellulose materials which comprises the addition of guanidine thiocyanates to an alkali metal formaldehyde-sulfoxylate discharge printing paste.

4. A preparation for the production of discharge effects on materials containing cellulose acetate comprising an alkali metal formaldehyde-sulfoxylate discharge printing paste and a guanidine thiocyanate.

5. A discharge composition for the class comprising cellulose esters and ethers containing a guanidine thiocyanate and a sulfoxylate.

6. A discharge composition for the class comprising cellulose esters and ethers containing an alkali metal formaldehyde sulfoxylate and a guanidine thiocyanate.

7. A discharge printing paste for cellulose acetate materials consisting of about 20 parts of sodium formaldehyde-sulfoxylate, about 55 parts of an approximately 6% gum tragacanth solution and about 25 parts of an approximately 50% guanidine thiocyanate solution.

8. A discharge printing paste for cellulose acetate materials comprising sodium formaldehyde-sulfoxylate, gum and guanidine thiocyanate. and ethers and thereafter discharging by ageing at about 100° C., washing and drying. 80
9. The production of discharge effects on materials of the class comprising cellulose esters and ethers which includes treatment with a guanidine thiocyanate. 10. The production of discharge effects on materials of the class comprising cellulose esters and ethers which includes treatment with guanidine thiocyanate. 11. The production of discharge effects on cellulose acetate materials which includes treatment with guanidine thiocyanate. 12. The process which comprises printing a discharge paste containing a guanidine thiocyanate on materials of the class comprising cellulose esters and ethers and thereafter discharging by ageing at about 100° C., washing and drying. 13. The process which comprises printing a discharge paste containing a guanidine thiocyanate on cellulose acetate materials and thereafter discharging by ageing at about 100° C., washing and drying. 14. The process which comprises printing a discharge paste containing an alkali metal formaldehyde-sulfoxylate and a guanidine thiocyanate on materials of the class comprising cellulose esters and ethers and thereafter discharging by ageing at about 100° C., washing and drying. 15. The process which comprises printing a discharge paste containing a guanidine thiocyanate on materials of the class comprising cellulose esters and ethers and thereafter discharging by ageing at about 100° C., washing and drying. 16. The process which comprises printing a discharge paste containing an alkali metal formaldehyde-sulfoxylate and a guanidine thiocyanate on cellulose acetate materials and thereafter discharging by ageing at about 100° C., washing and drying. 17. A discharge composition for the class comprising cellulose esters and ethers containing a guanidine thiocyanate and an alkali metal aldehyde sulfoxylate. 18. Dyed cellulose acetate material having imprinted thereon a discharge composition containing a guanidine thiocyanate and a sulfoxylate. 19. The process which comprises printing on a dyed cellulose acetate material a discharge composition containing an alkali metal aldehyde sulfoxylate and a guanidine thiocyanate and thereafter aging the imprinted material. 100
- FREDERICK B. DOWNING.  
RICHARD G. CLARKSON.
- 30 105
- 35 110
- 40 115
- 45 120
- 50 125
- 55 130
- 60 135
- 65 140
- 70 145
- 75 150